

## UNITED STATES PATENT OFFICE

2,050,197

PREVENTION OF DETERIORATION OF  
COTTON CORD BY HEATLorin B. Sebrell, Silver Lake, Ohio, assignor to  
Wingfoot Corporation, Wilmington, Del., a  
corporation of DelawareNo Drawing. Application March 10, 1932,  
Serial No. 598,098

2 Claims. (Cl. 8—20)

My invention relates to the treatment of cotton cord and to enhance its tensile strength and to enable it to maintain the same at temperatures of the order of those encountered in pneumatic tires under service conditions. The invention includes the method of treatment and the treated cotton material.

It has been observed heretofore that cords and threads, especially those prepared from cotton fibers, exhibit under X-rays a definite pattern associated with the molecular structure of the cotton. When subjected to moderate temperatures, for example, 250 degrees F., a molecular rearrangement occurs which causes the pattern to disappear, such rearrangement being accompanied by premature loss of strength and resultant failure of the cord or thread upon the application of relatively small tensional forces. Upon cooling, the major portion of the original strength is regained.

This loss of strength at high temperatures is particularly objectionable in cords employed in the construction of pneumatic tires, because much heat is developed in the latter when run at high speeds. In truck and bus tires, the temperatures sometimes reach values in excess of 250 degrees F. As a result, the cords of which the tire carcasses are composed and which normally are the principal tension resisting elements in the tire are so weakened that premature ruptures or blowouts tend to occur.

My invention resides in the discovery that ordinary cotton cords, threads, filaments, etc., when treated with reagents of the type herein described, continue to produce a definite X-ray pattern at temperatures materially above that at

which the pattern normally vanishes. Such treated cords also possess substantially greater tensile strength at ordinary temperatures and retain their original tensile strength when subjected to relatively high temperatures materially better than ordinary untreated cord. Although numerous reagents have been found more or less effective in retarding or resisting the action of high temperatures in cords, I have established by experiment that certain organic compounds, among which are the phenols, acids and aldehydes, are particularly effective.

The following are a few of the compounds which have been found satisfactory for the purposes mentioned.

|                    |    |
|--------------------|----|
| Phthalic acid      |    |
| Tannic acid        |    |
| Gallic acid        |    |
| Acetic acid        | 20 |
| Phenol             |    |
| Cresol             |    |
| Hydroquinone       |    |
| p-Hydroxy diphenyl |    |
| p-Nitroso phenol   | 15 |
| Pyrogallol         |    |
| Butyraldehyde      |    |
| Benzaldehyde       |    |
| Crotonaldehyde     | 10 |
| Heptaldehyde       |    |
| Aldol aldehyde     |    |
| Furfuraldehyde     |    |
| Formaldehyde       | 30 |

The results obtained with these compounds may be tabulated as follows:

| 40  | Chemical           | Chemical treatment                                                                                                                                                                                                                                                                                                                                          | Tensile of treated cord |        | Tensile of raw cord |        | 40 |
|-----|--------------------|-------------------------------------------------------------------------------------------------------------------------------------------------------------------------------------------------------------------------------------------------------------------------------------------------------------------------------------------------------------|-------------------------|--------|---------------------|--------|----|
|     |                    |                                                                                                                                                                                                                                                                                                                                                             | 250° F.                 | 75° F. | 250° F.             | 75° F. |    |
| 45  | Phthalic acid..... | 3 hrs. in 10% phthalic acid in alcohol at 70° C., allowed to stand in liquid 18½ hrs., dried at room temperature.<br>(a) 3 hrs. in 10% tannic acid in alcohol at 70° C., allowed to stand in liquid 18½ hrs., dried at room temperature.<br>(b) 2 hrs. in 20% tannic acid in water at 200° F., washed with 20% NaOH, extracted with benzene.                | 9.4                     | 19.3   | 10.7                | 17.5   | 45 |
|     | Tannic acid.....   | (a) 3 hrs. in 10% tannic acid in alcohol at 70° C., allowed to stand in liquid 18½ hrs., dried at room temperature.<br>(b) 2 hrs. in 20% tannic acid in water at 200° F., washed with 20% NaOH, extracted with benzene.                                                                                                                                     | 13.3                    | 20.9   | 10.7                | 17.5   |    |
| 50  | Gallic acid.....   | 3 hrs. in 10% gallic acid in alcohol at 70° C., allowed to stand in liquid 18½ hrs., dried at room temperature.<br>(a) 3 hrs. in 25% acetic acid in water at 70° C., allowed to stand in liquid 18½ hrs., dried at room temperature.<br>(b) 3 hrs. in 25% acetic acid in alcohol at 70° C., allowed to stand in liquid 18½ hrs., dried at room temperature. | 11.7                    | 19.8   | 10.7                | 17.5   | 50 |
|     | Acetic acid.....   | (a) 3 hrs. in 25% acetic acid in water at 70° C., allowed to stand in liquid 18½ hrs., dried at room temperature.<br>(b) 3 hrs. in 25% acetic acid in alcohol at 70° C., allowed to stand in liquid 18½ hrs., dried at room temperature.                                                                                                                    | 11.2                    | 17.1   | 10.7                | 17.5   |    |
| 55. |                    |                                                                                                                                                                                                                                                                                                                                                             | 12.6                    | 19.5   | 10.7                | 17.5   | 55 |

| 5  | Chemical                | Chemical treatment                                                                                                                                                                                                                                                                                                                                                              | Tensiles of treated cord |        | Tensiles of raw cord |        | 5  |
|----|-------------------------|---------------------------------------------------------------------------------------------------------------------------------------------------------------------------------------------------------------------------------------------------------------------------------------------------------------------------------------------------------------------------------|--------------------------|--------|----------------------|--------|----|
|    |                         |                                                                                                                                                                                                                                                                                                                                                                                 | 250° F.                  | 75° F. | 250° F.              | 75° F. |    |
| 10 | Cresol.....             | 3 hrs. in 25% cresol in alcohol at 70° C., allowed to stand in liquid 18½ hrs., dried at room temperature.                                                                                                                                                                                                                                                                      | 12.0                     | 19.8   | 10.7                 | 17.5   |    |
| 10 | Hydroquinone.....       | 3 hrs. in 25% hydroquinone in alcohol at 70° C., allowed to stand in liquid 18½ hrs., dried at room temperature.                                                                                                                                                                                                                                                                | 11.9                     | 20.4   | 10.7                 | 17.5   | 10 |
| 15 | p-Hydroxy diphenyl..... | 3 hrs. in 25% p-hydroxy diphenyl in alcohol at 70° C., allowed to stand in liquid 18½ hrs., dried at room temperature.                                                                                                                                                                                                                                                          | 11.8                     | 19.2   | 10.7                 | 17.5   |    |
| 15 | p-Nitroso phenol.....   | 3 hrs. in 10% p-nitroso phenol in alcohol at 70° C., allowed to stand in liquid 18½ hrs., dried at room temperature.                                                                                                                                                                                                                                                            | 11.5                     | 19.3   | 10.7                 | 17.5   | 15 |
| 20 | Pyrogallol.....         | 3 hrs. in 25% pyrogallol in alcohol at 70° C., allowed to stand in liquid 18½ hrs., dried at room temperature.                                                                                                                                                                                                                                                                  | 11.6                     | 19.1   | 10.7                 | 17.5   |    |
| 20 | Butyraldehyde.....      | Soaked 22½ hrs. in butyraldehyde at room temperature, heated 4 hrs. in liquid at 70° C., drained, dipped in alcohol, dried.                                                                                                                                                                                                                                                     | 12.6                     | 20.8   | 10.6                 | 17.6   |    |
| 25 | Benzaldehyde.....       | Soaked 22½ hrs. in benzaldehyde at room temperature, heated 4 hrs. in liquid at 70° C., drained, dipped in alcohol, dried.                                                                                                                                                                                                                                                      | 12.3                     | 19.7   | 10.6                 | 17.6   | 20 |
| 25 | Crotonaldehyde.....     | (a) Soaked 22½ hrs. in crotonaldehyde at room temperature, heated 4 hrs. in liquid at 70° C., drained, dipped in alcohol, dried.<br>(b) 2 hrs. in 100% dibutyl amine at 220° F., 3 hrs. in crotonaldehyde at 240° F.<br>(c) 3 hrs. in 100% dibutyl amine at 218° F., 3 hrs. in 20% crotonaldehyde in alcohol at 172° F.                                                         | 12.3                     | 20.2   | 10.6                 | 17.6   | 25 |
| 30 | Heptaldehyde.....       | (a) Soaked 22½ hrs. in heptaldehyde at room temperature, heated 4 hrs. in liquid at 70° C., drained, dipped in alcohol, dried.<br>(b) 3 hrs. in di-butyl amine (100%) at 198° F., 1½ hrs. in 20% heptaldehyde in alcohol at 174° F.<br>(c) 3 hrs. in 100% di-butyl amine at 218° F., 3 hrs. in 20% heptaldehyde in alcohol at 174° F., 100% carbon bisulphide.                  | 12.9                     | 20.9   | 10.6                 | 17.6   | 30 |
| 35 | Aldol aldehyde.....     | Soaked 22½ hrs. in aldol aldehyde at room temperature, heated 4 hrs. in liquid at 70° C., drained, dipped in alcohol, dried.                                                                                                                                                                                                                                                    | 11.1                     | 10.8   | -----                | -----  | 35 |
| 40 | Furfuraldehyde.....     | (a) Soaked 22½ hrs. in furfuraldehyde at room temperature, heated 4 hrs. in liquid at 70° C., drained, dipped in alcohol, dried.<br>(b) 3 hrs. in 100% dibutyl amine at 198° F., 1½ hrs. in 20% furfuraldehyde in alcohol at 174° F.<br>(c) 3 hrs. in 100% piperidine at 212° F., 1½ hrs. in 20% furfuraldehyde in alcohol at 174° F.                                           | 12.6                     | 20.5   | 10.6                 | 17.6   | 40 |
| 45 | Formaldehyde.....       | (d) 3 hrs. in 100% furfuraldehyde at 76° C.<br>(e) Heated gradually 1½ hrs. in 20% formaldehyde in water to 75° C., 2½ hrs. in liquid at 75° C., dried at room temperature.<br>(f) 3 hrs. in di-ethanol amine at 75° C., dried, 3 hrs. in 40% formaldehyde in water at 75° C.<br>(g) 3 hrs. in 40% formaldehyde in water at 75° C., dried, 3 hrs. in di-ethanol amine at 75° C. | 11.7                     | 10.8   | -----                | -----  | 45 |
| 50 |                         | (h) 3 hrs. in 40% formaldehyde in water at 75° C., dried, 3 hrs. in di-ethanol amine at 75° C.<br>(i) 3 hrs. in aniline, drained, 3 hrs. in 30% formaldehyde at 90° C.<br>(j) 3 hrs. in 25% phenol in water at 90° C., drained, 3 hrs. in 30% formaldehyde.                                                                                                                     | 12.1                     | 10.8   | -----                | -----  |    |
| 55 |                         | (k) 3 hrs. in 20% sodium phenolate, drained, 3 hrs. in 30% formaldehyde at 95° C.<br>(l) 3 hrs. in 85% diethyl amine at boiling point, 3 hrs. in 30% formaldehyde at 90° C.                                                                                                                                                                                                     | 11.7                     | 10.6   | -----                | -----  | 55 |
| 60 |                         |                                                                                                                                                                                                                                                                                                                                                                                 | 10.6                     | 17.3   | 10.1                 | 17.2   |    |
| 65 |                         |                                                                                                                                                                                                                                                                                                                                                                                 | 11.0                     | 18.7   | 10.1                 | 17.2   |    |
| 65 |                         |                                                                                                                                                                                                                                                                                                                                                                                 | 11.1                     | 18.3   | 10.1                 | 17.2   | 60 |
| 70 |                         |                                                                                                                                                                                                                                                                                                                                                                                 | 11.8                     | 18.1   | 10.1                 | 17.2   |    |
| 75 |                         |                                                                                                                                                                                                                                                                                                                                                                                 | 12.7                     | 19.0   | 10.1                 | 17.2   |    |
| 75 |                         |                                                                                                                                                                                                                                                                                                                                                                                 | 11.5                     | 18.7   | 10.1                 | 17.2   | 70 |
| 75 |                         |                                                                                                                                                                                                                                                                                                                                                                                 | 11.2                     | 17.4   | 10.1                 | 17.2   |    |
| 75 |                         |                                                                                                                                                                                                                                                                                                                                                                                 | 12.5                     | 19.5   | 10.1                 | 17.2   | 55 |

In these tests, samples of cord were treated with the several reagents mentioned, after which one set of samples was tested for tensile strength at normal or approximately room temperatures and at 34 percent relative humidity. The second set of samples was then subjected to tests identical with those conducted upon the first set, except that the temperature was maintained at a value of 250 degrees F. during the test. The con-

trol employed was identical in every respect with the treated cord, except that it was not treated.

From the table, it will be apparent that cords which have been treated are materially higher in tensile strength both at elevated temperatures and at ordinary or normal temperatures. In some cases, this increase amounts to as much as 30 percent to 40 percent at temperatures of 250 degrees. This increase is very advantageous in

case the cords are employed in bus tires or similar tires of large size which are run at relatively high speeds.

It will be apparent that my invention is not limited to cords employed in pneumatic tires. It may be used in connection with substantially any cotton fabric which is exposed to relatively high temperatures, one particular application being in connection with fabric employed in the manufacture of hose used to convey heated liquids. It is also to be understood that the invention is not limited to the specific compounds disclosed herein. All phenols, acids and aldehydes tested have been found to be effective to some extent, from which it appears probable that all such compounds exhibit properties of the kind described. In the claims hereof, these substances are referred to generically as acidic materials.

This application is a continuation in part of my prior application Serial No. 520,173, filed March 4, 1931, for Prevention of deterioration of cotton cord by heat now abandoned. Although I have described only the preferred forms which the invention may assume, it will be apparent to

those skilled in the art that it is not limited thereto, but that various modifications may be made therein without departing from the spirit of the invention or from the scope of the appended claims. It is intended that the patent shall cover, by suitable expression in the appended claims, whatever features of patentable novelty reside in the invention. 5

What I claim is:

1. A cotton cord treated with gallic acid, which 10 treated cord has the same general appearance and feels substantially the same as an untreated cotton cord and has greater tensile strength at 250° F. than the untreated cord at the same temperature. 15

2. The method of preserving the tensile strength of cotton cord under conditions of heat which comprises applying gallic acid thereto, whereby without substantial chemical action on the cotton of the cord, the cord is made to have 20 greater tensile strength at 250° F. than the untreated cord at the same temperature.

LORIN B. SEBRELL.